

Aug. 2, 1960

G. LANDELLS ET AL

2,947,058

ORNAMENTATION OF SHEET MATERIAL

Filed Feb. 7, 1956



Inventors  
GEORGE LANDELLS  
WILLIAM BRAGG  
By  
Mead, Bowes, Schuyler, Beveridge  
Attorneys

1

2,947,058

## ORNAMENTATION OF SHEET MATERIAL

George Landells, Leeds, and William Bragg, West Ardsley, near Wakefield, England, assignors to The Bradford Dyers' Association Limited, Bradford, and Bleachers' Association Limited, Manchester, England

Filed Feb. 7, 1956, Ser. No. 564,081

Claims priority, application Great Britain Feb. 10, 1955

9 Claims. (Cl. 26—69)

This invention relates to the ornamenting of compressively shrinkable sheet materials such as fabrics, films, foils or the like. It is well known that fabrics can be compressively shrunk by being subjected to pressure applied both normally and lengthwise of the fabric. Other sheet materials capable either of being forced to thicken or of being reduced in volume, and therefore contracted, can be compressively shrunk in the same way. In one well-known process of compressive shrinking the sheet material is pressed against a contractile surface, e.g. against a rubber belt, while that surface contracts, so that the material contracts with the surface. Such materials include, as well as fabrics, leather, regenerated cellulose and plastic sheets and coated textiles such as bookcloth, imitation leather cloth and the like.

It is an object of the present invention to ornament compressively shrinkable sheet material by changing the configuration of the material by the random formation of buckles, crinkles or the like.

It is a further object of the invention to compressively shrink sheet material and at the same time to form an ornamentation thereon.

A compressively shrinkable sheet material is ornamented in accordance with this invention by compressively shrinking the material in contact with a second buckable sheet material so that the buckles formed in the second material are transferred to the first material. The invention is particularly applicable to the ornamentation of fabrics; the second sheet material may advantageously be paper.

The nature of the effect produced on a fabric under given conditions with the same second sheet material depends on the fabric under treatment. Fabrics possessing smooth shiny surfaces, such as satins or sateens, respond particularly well. Fabrics may be prepared for the process with advantage by calendering or pressing to produce a smooth or glossy surface. The effect produced varies from a random distribution of coarse buckles or pockers, running generally across the width of the material, to finer buckles or ripples.

The material which buckles is generally stiffer than the compressively shrinkable sheet material, and although it may shrink slightly before it starts to buckle, this is unimportant so long as some buckling takes place. For instance, some paper will shrink by 1 or 2% but thereafter will buckle. The shrinking conditions must be such that the compressively shrinkable sheet material not only shrinks but accepts the buckles and that the second sheet material buckles. If the first material is treated along under the shrinking conditions in question, it will shrink but not buckle, whereas the second material treated alone will buckle.

The ornamentation is resistant to normal handling but may be largely or wholly lost on wetting or washing the material unless steps are taken to fix it. Such a step

2

is the pre-treatment of the material with an agent which will set by heat applied during or after the ornamenting, or by the action of a chemical reagent applied after the ornamenting and setting the agent or bringing about a reaction with the chemical reagent to maintain the ornamentation.

If the compressively shrinkable material is of nylon, a polyethylene terephthalate or other thermoplastic which when deformed while heated will retain its deformed shape until it is heated to a higher temperature the ornamentation is advantageously fixed by heating the material to an appropriate heat-setting temperature during the ornamenting, the effect of the heating being to fix or stabilize the ornamentation against mechanical action at a temperature lower than that reached during the treatment.

For example a cotton fabric may be impregnated with a thermosetting resin in aqueous solution and then dried. It is then ornamented according to the invention and heated at a temperature to complete the condensation of the resin, thus fixing the ornamentation. Preferably, one of the rollers or other elements of the shrinking apparatus is heated to a temperature sufficient to set the resin used, but the time of contact with the heated roller is usually insufficient to complete the condensation and an additional heating step is then required. Even thermoplastic materials may also be subjected to this resin treatment, having the effect in this instance of stiffening the material rather than fixing the ornamentation.

Where the material is composed wholly of cellulose acetate or contains a high proportion of cellulose acetate, the material may be temporarily plasticised by water or solutions of swelling agents to render the material more amenable to the ornamenting process. The plasticiser must not, of course, interfere with the buckling properties of the second sheet material.

The invention will now be described in greater detail by reference to the accompanying diagrammatic drawings in which:

Figures 1 and 2 are sectional views through two shrinking machines of different types operating according to this invention;

Figures 3 and 4 are views showing two different ornamentations obtained according to the invention.

Referring first to Figure 1, which shows the preferred machine for carrying out the invention, a thick endless rubber or equivalent belt 11 passes around two rollers 12 and 13, the fabric or other material 16 being fed on to the belt between it and a third roller 14 at a point in advance of that at which the surface of the belt begins to contract in reversing its curvature. The roller 14 can be adjusted in the direction of the arrows C to vary the pressure between the roller and the belt. Movement can be imparted to the belt by driving any of the three rollers. The second sheet material 17 is also fed into the nip between the belt 11 and the roller 14 on the side of the material remote from the belt. It can be fed between the fabric or the like and the belt, but this is not generally so effective. The second sheet material 17 is fed into the nip between the roller 14 and the belt 11 from a roll 15 and passes around the roller 14 under tension. If the material 17 is fed directly to the nip as shown by the dotted line 17' there is a tendency for the material to crease as it enters the nip, forming undesirable markings on the material 16.

It is well known that the degree of shrinkage imparted by a compressive shrinking machine to a fabric can be varied, particularly by varying the pressure, temperature or moisture content, and therefore the ornamentation can be varied. The greater the pressure, the more numerous

and smaller are the buckles produced. Naturally the actual number of buckles produced under given conditions depends on the nature and stiffness of the second material. It is not only the pressure but also the temperatures that must be appropriately adjusted. For instance, in treating one cellulose acetate fabric and paper together under a given pressure, substantially no ornamentation was produced at 200° F. but a good crinkled effect was produced at 275° F. Figures 3 and 4 show two different ornamentations obtained in the apparatus shown in Figure 1. The general surface of the material remains flat, but buckles 18 are formed. These are transferred from the second sheet material.

Figure 2 shows a machine of the kind in which there is a narrow passage between a roller and a curved bed plate and the material to be shrunk is fed into this passage at a higher speed than it is allowed to emerge. In the machine illustrated a roller 20 and an electrically heated bed plate 21 form a feed nip and another roller 22 cooperates with the first to form an outlet nip. The compressively shrinkable sheet material 23 and the second sheet material 24 are fed into the inlet nip over a rail 25 and then pass to the passage 26 finally leaving the machine through the outlet nip. The roller 20 has a hard rubber surface and rotates at a faster speed than the roller 22 which has a soft rubber surface. The width of the passage is adjusted by moving the rollers 20 and 22 in the direction of the arrows A and B.

While we have described and illustrated two particular compressive shrinking machines for use in this invention any other type or construction of machine may also be used.

In a variation of the invention the compressively shrinkable sheet material is compressively shrunk in contact with a third sheet material which also buckles, such as that shown by broken line 24' in Fig. 2, the third sheet material being on the opposite side of the first sheet material from the second sheet material. The third material may or may not be the same as the second.

The compressively shrinkable sheet material may be subjected to two separate ornamenting processes, the conditions in each process preferably being different, so that two ornamental effects are superimposed on each other.

Instead of using paper as the second sheet material we may use cardboard, a plastic, thin sheet metal, a fabric stiffened by a resin, starch or other stiffening agent, or even a fabric so woven that it will not readily shrink, but rather tends to buckle, if compressively shrunk alone.

If either of the surfaces between which the two materials are pressed during the treatment is discontinuous the compressive shrinking is discontinuous over the surface of the compressively shrinkable sheet material and ornamentation according to the invention takes place only in selected areas. The remaining areas which are not compressively shrunk will form ruffles, frills, puckers or the like between the compressively shrunk areas.

The sheet material which buckles may be discontinuous or have an embossed surface. In the first case no buckles will be formed in those areas not in contact with the second sheet material and in the second case the buckles will be superimposed on an embossed design.

Some examples will now be given.

#### Example 1

A piece of polyvinyl chloride sheet (.005" thick) was superimposed on a sheet of paper card (.009" thick) and the two materials introduced into the nip of a machine of the type shown in Figure 1. The paper card was in contact with the roller 14 which was heated to 190° F. Passage through the machine caused buckling of the paper card, buckles being transferred to the plastic sheet, which also shrank slightly.

The plastic sheet did not buckle when passed through the machine alone.

#### Example 2

5 A piece of black skin leather (thickness 0.04") having one surface polished and the reverse matt, was introduced into the nip of a machine of the type shown in Figure 1 together with a sheet of glazed kraft paper (0.005" thick). The polished surface of the leather was in contact with the paper, the paper being in contact with the roller 14. This roller was heated to 280° F. Since the paper possessed little or no contractile property, passage through the shrinking machine caused lateral crinkles to occur randomly distributed throughout the paper. These crinkles were transferred to the leather which also shrank 7.5%.

#### Example 3

15 The roller 14 of a compressive shrinkage machine of the type shown in Figure 1 was heated to 340° F. The roller was pressed against the rubber belt 11 and a test length of paper 0.003 inch thick passed through the machine. The paper shortened, essentially by buckling, by 8½%. A cellulose acetate satin fabric was led from a roll and superimposed on a paper sheet of the same material as the test length, also delivered from a roll so that the satin face of the fabric was adjacent to the paper. The two sheet materials were led between the roller 14 and the belt 11 with the paper next to the roller. Shortening and buckling of the paper took place and the numerous buckles were simultaneously reproduced in the satin fabric to give an attractive decorative effect. The fabric was found to have shrunk by 9½%.

#### Example 4

20 A specimen of a plain weave cotton fabric was impregnated with a solution of 7.5 parts (all parts are by weight) of a methylated trimethylol melamine precondensate and 0.5 part of ammonia dihydrogen phosphate in 92 parts of water and mangled to contain 90 parts of the solution for every 100 parts of fabric. The fabric was dried under conditions in which substantially no condensation took place and then treated as in Example 3. The ornamented fabric emerging from the machine was separated from the buckled paper and heated in a hot air oven for 3 minutes at 300° F. The ornamentation was thus rendered resistant to repeated washing in a soap solution.

#### Example 5

25 A cellulose acetate satin fabric was fed into the passage between the roller 20 and the bedplate 21 of a machine of the type illustrated in Figure 2 together with paper 0.0025 inch thick, the paper being adjacent the bedplate. The bedplate was maintained at 250° F. The roller 20 was driven at a surface speed of 11.7 feet per minute and the roller 22 at a surface speed of 6.0 feet per minute. The satin fabric emerging from the confining passage carried innumerable small lateral ripples. The satin fabric was passed through the machine alone and it shrank, but no ornamentation was obtained.

30 We claim:

1. An ornamenting process in which ornamental buckles are formed in a compressively shrinkable sheet material which comprises compressively shrinking said material while in surface contact with a compressively bucklable sheet material on each side of said compressively shrinkable sheet material.
2. An ornamenting process in which ornamental buckles are formed in a compressively shrinkable sheet material which comprises compressively shrinking said material while in surface contact with a compressively bucklable sheet material in selected areas over the surface of said compressively shrinkable sheet material.
3. A process for ornamenting compressively shrinkable sheet material which normally shrinks but does not buckle when subjected to the action of a compressive shrinking machine, which process comprises producing

ornamental buckles in the shrinkable sheet material by subjecting said material to the action of a compressive shrinking machine while in surface contact with compressively bucklable sheet material which normally buckles when subjected to the action of a compressive shrinking machine.

4. A process according to claim 3 wherein the compressively shrinkable sheet material is a fabric.

5. A process according to claim 3 wherein the compressively shrinkable sheet material is leather.

6. A process according to claim 3 wherein the compressively shrinkable sheet material is polyvinyl chloride.

7. A process for ornamenting compressively shrinkable sheet material which normally shrinks but does not buckle when subjected to the action of a compressive shrinking machine, which process comprises producing ornamental buckles in the shrinkable sheet material by subjecting said material to the action of a compressive shrinking machine while in surface contact with compressively bucklable sheet material which normally buckles 20

when subjected to the action of a compressive shrinking machine, and treating the shrinkable sheet material to retain the ornamental buckles.

8. A process according to claim 7 wherein the compressively shrinkable material is thermoplastic.

9. A process according to claim 7 wherein the compressively shrinkable sheet material is polyvinyl chloride.

References Cited in the file of this patent

UNITED STATES PATENTS

|    |           |                |                |
|----|-----------|----------------|----------------|
| 10 | 1,643,147 | Angier         | Sept. 20, 1927 |
|    | 2,078,904 | Glueett        | Apr. 27, 1937  |
|    | 2,079,273 | Angier         | May 4, 1937    |
| 15 | 2,146,694 | Wrigley et al. | Feb. 7, 1939   |
|    | 2,667,910 | Grettve        | Feb. 2, 1954   |
|    | 2,825,117 | Evans et al.   | Mar. 4, 1958   |

FOREIGN PATENTS

|               |         |               |
|---------------|---------|---------------|
| Australia     | 165,590 | Oct. 13, 1955 |
| Great Britain | 376,040 | July 7, 1932  |